

# UNITED STATES PATENT OFFICE.

HENRY F. H. MILLER, OF BOSTON, MASSACHUSETTS.

## IMPROVEMENT IN WATER-PROOF COMPOUNDS.

Specification forming part of Letters Patent No. 178,319, dated June 6, 1876; application filed November 27, 1875.

*To all whom it may concern:*

Be it known that I, HENRY F. H. MILLER, of Boston, in the county of Suffolk and State of Massachusetts, have invented certain new and useful Water-Proof Boot and Shoe Polishing Wax; and I do hereby declare that the following is a full, clear, and exact description thereof, which will enable others skilled in the art to which it pertains to make and use the same.

My invention relates to a new article of manufacture for the purpose of polishing boots and shoes, &c., without the need of a brush. By the use of this my invention the leather is rendered very soft, glossy, and pliable, and preserved from decay, as well as rendered water-proof and water-repelling.

This my invention is molded in a convenient shape, so as to be carried in one's pocket, if required, without soiling the same, and, as a dressing, it is particularly applicable to boots and shoes in moist and damp weather, when it will protect the feet thoroughly from dampness.

The manner in which my invention is used is simply to rub the wax lightly over the boot or shoe, and then to rub or polish it gently with a cloth of any suitable material, although cotton cloth is preferable for this purpose. Boots or shoes dressed and polished with my invention may be exposed to dampness and water without affecting the polish thereon, or

allowing the moisture and water to penetrate the same.

My invention is composed and made as follows: About ten pounds of paraffine-wax, six pounds of stearic acid, and four pounds of beeswax are heated and melted together in a suitable vessel. I then add about two pounds of ivory-black, one and one half pound of lamp-black, three ounces of gum-dammar, ten ounces of pulverized sugar, one-half gill of high-proof alcohol, one-half gill of spirits of turpentine, and three ounces of bar-soap.

The above is kept stirred while being brought to boiling, and also when it is put into suitable molds, after which it is allowed to cool, and is then ready for use.

What I claim, and wish to secure by Letters Patent, is—

The water-proof boot and shoe polishing wax, as herein described, composed of paraffine-wax, stearic acid, beeswax, ivory-black, lamp-black, gum-dammar, sugar, alcohol, spirits of turpentine, and bar-soap, in or about the proportions specified.

In testimony that I claim the foregoing as my own invention I have affixed my signature in presence of two witnesses.

HENRY F. H. MILLER.

Witnesses:

ALBAN ANDRÉN,  
SARAH M. MILLER.